

May 19, 1925.

1,537,950

L. KIRSCHBRAUN

WATERPROOF COVERING AND PROCESS OF MAKING SAME

Original Filed Feb. 1, 1919



witness:

*Stephen H. Kirschbraun*

Inventor:  
Lester Kirschbraun,  
by Frank L. Belknap,  
*Hatty*

Patented May 19, 1925.

1,537,950

# UNITED STATES PATENT OFFICE.

LESTER KIRSCHBRAUN, OF EVANSTON, ILLINOIS.

## WATERPROOF COVERING AND PROCESS OF MAKING SAME.

Application filed February 1, 1919; Serial No. 274,496. Renewed October 28, 1921. Serial No. 511,099.

To all whom it may concern:

Be it known that I, LESTER KIRSCHBRAUN, a citizen of the United States, residing in the city of Evanston, county of Cook, and State of Illinois, have invented certain new and useful Improvements in Waterproof Coverings and Processes of Making Same, of which the following is a specification.

This invention relates to the manufacture 10 of waterproof coverings, and is especially adapted for use as an ornamental waterproof flooring, similar to printed linoleums; to provide a product of the above character in which the upper surface of the floor covering is suitably ornamented and in which, 15 the body portion is waterproof; to provide a product in which a water resisting sealing layer is interposed between the upper ornamentation and the body portion; to provide 20 a process in which the above product is formed as a continuous and simultaneous operation, and, in general, to provide improvements of the character referred to.

In the manufacture of ornamental flooring felts, the body portion is made of paper felt saturated with black asphalt or bitumen. The colored ornamentation is painted over this saturated felt, and several layers of paint are required in order to prevent the 25 black bitumen from discoloring the ornamentation. This process is slow and expensive, first, because a relatively thick layer of paint must be used, and, secondly, because each coat must be thoroughly dry before the next one is applied. The present 30 invention obviates the above difficulty. The waterproof body portion and the sealing layer are formed simultaneously, and the ornamentation can then be applied with the 35 minimum amount of paint.

The single figure of the drawing is a cross-sectional elevational view of the finished sheet.

The invention may be carried on as follows:

An aqueous mixture of clay containing a sufficient percentage of colloidal particles, or an analogous emulsifying agent, is first made. While this mixture is in heated condition a binder, in liquid form, is added to the aqueous mixture and thoroughly dispersed therethrough so as to form an emulsion in which the emulsifying agent and aqueous vehicle form the external phase and the binder the internal phase. The binder 50 may be either asphalt, linseed oil or other

suitable ingredient. This emulsified matrix may consist, by weight, of fifty parts binder, ten parts clay and forty parts water. This emulsified matrix is then mixed with the fibre contained in an aqueous vehicle so as to thoroughly commingle the fibre with the emulsion. The matrix and fibre may be mixed in the ordinary beater, such as used in paper mills. In another beater paper stock, suitably sized, is formed in the ordinary way. The amount of size and character is varied with the end in view of producing a highly water-resistant paper. The two mixtures are then run over a multiple cylinder machine so that the waterproof body portion is formed in a sheet with the water-resistant sized paper, forming a layer affixed to the body portion. The sheet formed in this way, after being dried, is ready to receive a ground paint coat, and the ornamentation can then be applied. It is to be noted that in the formation of the above sheet as the water dries out of the body portion the emulsion is broken and the adhesive 60 binder intimately unites with the fibre. Also that the body portion is permanently attached to the sized outer layer portion. In certain cases, in order to obtain resiliency for the flooring, it may be desirable to add 65 to the body portion comminuted cork or sawdust. This can be mixed with the fibre in the beater either before or after the matrix is added.

The applicant in this application is not 70 claiming broadly the process of making emulsion, or the product produced thereby, or broadly covering the idea of mixing such emulsified product with fibre, the same being claimed in other co-pending applications of 75 this applicant.

I claim as my invention:

1. A process of making an ornamental waterproof covering, consisting in forming a mixture of fibre and a bituminous emulsified matrix into a sheet, simultaneously forming sized paper stock into an outer ply portion, bringing together the plies drying out the water and allowing the bitumen to intimately unit with the fibre, and the plies 100 to intimately unite together, and then painting an ornamentation on the outer ply.

2. A process of making a waterproof sheet on a paper machine, consisting in sheeting a mixture of fibre and a bituminous emulsion, simultaneously forming sized paper stock into an outer ply portion, bringing to- 105

gether the plies drying out the water and allowing the bitumen to intimately unite with the fibre, and the plies to intimately unite together.

5. 3. A waterproof sheet, consisting of multiple plies, comprising a body portion formed of fibre, emulsifying agent, an adhesive binder, and an outer portion formed of sized paper stock, the two portions being intimately united and having the structure characteristics of being simultaneously formed.
10. 4. A waterproof covering sheet, consisting of multiple plies, comprising a body portion formed of fibre, emulsifying agent, and an adhesive binder, and an outer portion formed of sized paper stock, the two portions being intimately united and having the structural characteristics of having been simultaneously formed, and an ornamentation applied to the outer sheet portion.
15. 5. A waterproof covering sheet consisting of multiple plies comprising a body portion formed of fibre, an emulsifying agent, and a bituminous binder and an outer portion formed of paper stock, the two portions being intimately united and having the characteristics of being simultaneously formed.
20. 6. A waterproof covering sheet consisting of multiple plies comprising a body portion formed of fibre, and an emulsifying agent, a bituminous binder, an outer portion formed of paper stock, the two portions being intimately united and having the characteristics of having been simultaneously

formed and an ornamentation applied to the outer portion.

7. A waterproof covering consisting of multiple plies comprising a body portion formed of fibre, an emulsifying agent and asphalt, and an outer portion formed of paper stock, the two portions being intimately united during formation.

8. A waterproof covering consisting of multiple plies comprising a body portion formed of fibre, an emulsifying agent and asphalt, and an outer portion formed of paper stock, the two portions being intimately united during formation, and an applied ornamentation on the outer portion.

9. A process of making a waterproof sheet on a paper machine, consisting in forming a mixture of fibre and a bituminous emulsion into a body portion, simultaneously forming a fibrous stock into an outer ply portion, uniting the outer ply to one surface of the body portion to form a unitary structure, drying the sheet and allowing the bitumen to coalesce.

10. A waterproof sheet consisting of multiple plies comprising a body portion formed of fibre, emulsifying agent, an adhesive binder and comminuted resilient filler, and an outer portion formed of paper stock, the two portions being intimately united, and having the characteristics of being simultaneously formed.

LESTER KIRSCHBRAUN.